

[54] **METHOD FOR LOCATING THE  
REMAINING RECOVERABLE MINERAL  
RESERVES DURING SOLUTION MINING**

[75] Inventor: Dennis E. Stover, Plano, Tex.

[73] Assignees: Atlantic Richfield Company, Los Angeles, Calif.; NM Uranium, Inc., Houston, Tex.; The United States Steel Corporation, Pittsburgh, Pa.

[21] Appl. No.: 864,352

[22] Filed: Dec. 27, 1977

[51] Int. Cl.<sup>2</sup> ..... E21B 43/28

[52] U.S. Cl. ..... 299/4

[58] Field of Search ..... 299/4, 5; 166/250, 252

[56] **References Cited**

**U.S. PATENT DOCUMENTS**

|           |        |               |       |
|-----------|--------|---------------|-------|
| 3,708,206 | 1/1973 | Hard et al.   | 299/5 |
| 3,713,698 | 1/1973 | Rhoades       | 299/4 |
| 3,860,289 | 1/1975 | Learmont      | 299/4 |
| 4,032,194 | 6/1977 | Howell et al. | 299/4 |

4,083,603 4/1978 Stover ..... 299/4

**OTHER PUBLICATIONS**

Sievert et al., "In Situ Leaching of Uranium", SME Preprint Number 70-AS-334, Oct. 1970.

*Primary Examiner*—Stephen J. Novosad  
*Assistant Examiner*—George A. Suchfield  
*Attorney, Agent, or Firm*—Ronnie D. Wilson

[57] **ABSTRACT**

The present invention relates to a method for the solution mining of a mineral from a subterranean formation. More specifically, the invention relates to a method which enhances significantly the recovery of a mineral from a subterranean formation via solution mining utilizing an oxidant and leach solution with an injection and production well. The method comprises ceasing oxidant injection via the injection well and measuring the change in mineral concentration in the pregnant solution recovered via the production well.

**8 Claims, No Drawings**

METHOD FOR LOCATING THE REMAINING  
RECOVERABLE MINERAL RESERVES DURING  
SOLUTION MINING

Generally, known methods for solution mining of a mineral in situ utilize an acid or alkaline leach solution for the dissolution of the mineral. An oxidant is injected into the formation along with the leach solution. The mineral is leached from the formation and recovered from a production well via a pregnant leach solution. Various procedures for recovering the mineral from the pregnant leach solution are well known, such as ion exchange.

The method of the present invention is particularly suitable for the leaching of uranium; however, my invention is not so limited. The following description of the present invention will be applied to uranium leaching; however, it is apparent that it is applicable to leaching other mineral values such as copper, nickel, molybdenum, rhenium and selenium where similar problems are encountered.

Although acid leaching solutions can be used in some formations, only alkaline leaching solutions can practically be used where the particular formation contains significant quantities of acid-consuming gangue.

It is well known that to recover uranium from an underground ore body, it is necessary to convert the relatively insoluble tetravalent state of uranium in the ore to the solubilizable hexavalent state. When using an alkaline leach solution, the dissolution of the uranium in solution occurs in two steps. The first step involves the oxidation of uranium by adsorbing oxygen and the second is the dissolution of the oxidized uranium in the solution.

During the early stages (when the ore body is in a reduced state) of a leach operation utilizing alkaline solutions of ammonium carbonate, sodium carbonate, potassium carbonate and their respective bicarbonates in conjunction with the typical oxidants of air, oxygen, and hydrogen peroxide, a portion of the uranium that is oxidized and dissolved near the injection well is reduced and precipitated in the more reduced regions of the formation between the injection well and the production well. Through this action the oxidized region of the formation is depleted of uranium and the reduced region of the formation becomes enriched as the leach operation continues. Therefore, this process of oxidation and dissolution followed by partial reduction and precipitation continues as the formation becomes progressively oxidized, whereby the region in the immediate vicinity of the production well becomes progressively enriched. As a result, the uranium is depleted from a zone in the formation far more quickly than the oxidant consuming gangue species present therein.

Therefore, as the uranium oxidation front recedes from the injection well, the oxidant available for uranium oxidation decreases. This causes a slower dissolution of uranium and a lower maximum concentration of uranium in solution as the depleted zone moves through the formation. The continued injection of oxidant and leach solution through an injection well away from which the uranium oxidation front has moved is wasteful, since most of the injected oxidant reacts with gangue material and leach solution contacts little oxidized uranium. Fluid produced from a production well in exclusive communication with such an injection well contains little or no uranium. In a multi-well configura-

tion, the fluid dilutes the uranium concentration from other wells and thereby decreases the efficiency of the operation. To conduct a solution mining operation efficiently and provide for maximum uranium recovery, it is necessary to focus the flow of oxidant and leachant on the remaining uranium reserves and to minimize the flow through depleted or barren areas of the formation. To achieve this, the location of the remaining uranium reserves must be known. Therefore, there is needed a method whereby the remaining reserves in a formation containing a mineral such as uranium can be located and recovered with a leach solution without being accompanied by excessive losses of oxidant and leach solution.

Therefore, it is an object of the present invention to provide a method for the solution mining of a mineral from a subterranean formation, applicable generally to minerals requiring oxidation to be leached and to both acid and alkaline leach solutions.

A further object of the present invention is to provide a method for the solution mining of uranium.

It is an additional objective of the present invention to provide a method for locating remaining reserves recoverable by solution mining from subterranean deposits.

Other objects, aspects, and the several advantages of the present invention will become apparent upon a further reading of this disclosure and the appended claims.

It has now been found that the objects of the present invention can be attained in the solution mining of mineral from a subterranean formation containing same where an injection and production well are drilled and completed within said formation, a leach solution and an oxidant are injected through the injection well into the formation to dissolve the mineral and recover it via a production well, by temporarily ceasing the injection of oxidant and measuring the change in mineral concentration in the solution recovered via the production well.

In the operation of the present invention to locate remaining recoverable uranium, the injection of oxidant into a given injection well is stopped while continuing leach solution injection for a period of time required to measure the change in uranium concentration in the pregnant leach solution recovered via the production well. By measuring the uranium concentration in the pregnant solution without oxidant injection, one can determine the relative uranium production contributed by a given injection well. Thus, the remaining recoverable uranium is located and steps taken to most efficiently utilize oxidant and leach solution to recover same.

Of course, the period of time which oxidant injection should be stopped will vary from formation to formation. Suitable dye tests can be made to determine more specifically the actual time needed to yield a good observation of the location of the reserves remaining.

The following illustrations will show the effective operation of the present invention.

1. When the ceasing of oxidant injection into an injection well produces no change in the uranium concentration of the pregnant solution recovered from an adjacent production well, the recoverable uranium in that area is completely oxidized. Thus, oxidant injection should be permanently stopped because continued injection merely oxidizes the gangue material present therein. Leach solution should continue to be injected to recover the oxidized uranium.

When the individual interruption of oxidant injection into four offset injection wells centered by a production well shows that three of the wells provide essentially all of the uranium production, the recoverable 5 nium has been depleted near the fourth well. The rth injection well should be abandoned for efficient ration.

By the testing of four offset injection wells centered by a production well via oxidant cessation, it is 10 found that the four injection wells are contributing to production of uranium in the order of 5, 15, 30 and 7% corresponding to each of the wells. Since the concentration of uranium in the pregnant solution is proportional to the remaining recoverable reserves, this 15 shows that the latter injection well has the largest amount of remaining recoverable reserves. By utilizing information obtained, an efficient strategy of final pper stage of operation can be developed.

Therefore, through the utilization of the present invention, the recovery of uranium via in situ leaching 20 processes can be enhanced significantly by most effectively using the oxidant and leach solution to recover remaining reserves present in the formation.

In addition, the present invention provides direct 25 measurements of the pattern performance under normal operating conditions, since the stream lines between injection and production wells remain constant during utilization.

Having thus described my invention, I claim:

1. A method for locating the remaining mineral reserves recoverable via solution mining from a subterranean formation containing said mineral in which an 30

injection and production well are drilled and completed within said formation, leach solution and an oxidant are injected through said injection well into said formation to dissolve said mineral, and said dissolved mineral is recovered via said production well, which comprises temporarily ceasing said injection of oxidant and measuring the change in mineral concentration in the solution recovered via said production well.

2. The method of claim 1 wherein said mineral is selected from the group consisting of copper, nickel, molybdenum, rhenium, selenium and uranium.

3. The method of claim 1 wherein said leach solution is acidic in nature.

4. The method of claim 3 wherein said acid leach solution is selected from the group consisting of hydrochloric and sulfuric acid.

5. The method of claim 1 wherein said leach solution is alkaline in nature.

6. The method of claim 5 wherein said alkaline leach solution is an aqueous solution of one or more salts selected from the group consisting of ammonium carbonate, sodium carbonate, potassium carbonate and their respective bicarbonates.

7. The method of claim 1 wherein said oxidant is selected from the group consisting of air, oxygen and hydrogen peroxide.

8. The method of claim 1 wherein said injection and said production well are arranged in a five spot pattern having one production well centered between four offset injection wells.

\* \* \* \* \*